

Nov. 6, 1962

S. B. HUDAK ET AL

3,062,693

METHOD OF IMPROVING IMPACT RESISTANCE OF MILD STEEL

Filed July 2, 1959

8 Sheets-Sheet 1



INVENTORS

STEPHEN B. HUDAK,  
WILLIAM C. LESLIE and  
REGINALD L. RICKETT

By Donald G. Dalton  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 2



FIG. 2 -- V-NOTCH CHARPY IMPACT RESISTANCE OF STEEL B (RIMMED, 0.10 % C )

INVENTORS  
STEPHEN B. HUDAK,  
WILLIAM C. LESLIE and  
REGINALD L. RICKETT  
By Donald G. Dalton  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 3



FIG. 3--V-NOTCH CHARPY IMPACT RESISTANCE OF STEEL C. (ALUMINUM-KILLED, 0.10% C)

INVENTORS

STEPHEN B. HUDAK,  
WILLIAM C. LESLIE and  
REGINALD L. RICKETT

By *Donald G. Dalton*  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 4



FIG. 4 -- V-NOTCH CHARPY IMPACT RESISTANCE OF STEEL C (ALUMINUM - KILLED, 0.10% C)

INVENTORS  
STEPHEN B. HUDAK,  
WILLIAM C. LESLIE and  
REGINALD L. RICKETT  
By Donald G. Dalton  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 5



FIG. 5 -- V - NOTCH CHARPY IMPACT RESISTANCE OF STEEL D ( ALUMINUM - KILLED, 0.10% C )

INVENTORS

STEPHEN B. HUDAK,  
WILLIAM C. LESLIE and  
REGINALD L. RICKETT

By *Donald G. Dalton* Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 6



FIG. 6 -- V-NOTCH CHARPY IMPACT RESISTANCE OF STEELS B (RIMMED) AND D (ALUMINUM KILLED) HEATED TO 1750 F, QUENCHED TO 1450 F, THEN AIR COOLED.

INVENTORS  
STEPHEN B. HUDAK,  
WILLIAM C. LESLIE and  
REGINALD L. RICKETT  
By Donald G. Dalton  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 7



FIG. 7 -- V-NOTCH CHARPY IMPACT RESISTANCE OF STEEL D (ALUMINUM-KILLED, 0.10% C)

INVENTORS  
STEPHEN B. HUDAK,  
WILLIAM C. LESLIE and  
REGINALD L. RICKETT  
By Donald G. Dalton  
Attorney

Nov. 6, 1962

S. B. HUDAK ET AL

3,062,693

METHOD OF IMPROVING IMPACT RESISTANCE OF MILD STEEL

Filed July 2, 1959

8 Sheets-Sheet 8



FIG. 8 -- V-NOTCH CHARPY IMPACT RESISTANCE OF STEEL I (0.21% C)

INVENTORS

STEPHEN B. HUDAK,  
WILLIAM C. LESLIE and  
REGINALD L. RICKETT

By *Donald G. Dalton*  
Attorney

1

3,062,693

METHOD OF IMPROVING IMPACT RESISTANCE  
OF MILD STEEL

Stephen B. Hudak, Pleasant Hills, and William C. Leslie and Reginald L. Rickett, Franklin Township, Westmoreland County, Pa., assignors to United States Steel Corporation, a corporation of New Jersey

Filed July 2, 1959, Ser. No. 824,590

9 Claims. (Cl. 148—134)

This invention relates to a method of improving the impact resistance of mild steel and more particularly to a method of lowering the notch impact transition temperature of such steel.

Brittle fractures in large steel structures, such as ships, storage tanks, bridges and the like have caused large and unexpected losses and have been the subject of intensive investigation of both users and manufacturers of mild steel. These investigations have shown that the notch impact properties of mild steels can be improved by deoxidizing with aluminum but for various reasons it is not desirable to use such "killed" steels for many purposes. It has also been determined that notch impact properties can be improved by increasing the manganese/carbon ratio which however considerably increases the steel cost.

It is accordingly an object of the present invention to provide an improved and efficient method of lowering the notch impact transition temperature of mild steel.

It is another object of this invention to provide a method of lowering the notch impact transition temperature of both killed and rimmed mild steels.

The foregoing and further objects will be apparent when read in conjunction with the attached drawings, wherein:

FIGURES 1 through 7 are graphs with accompanying photomicrographs showing the structure and notch impact properties of various steels after treatment in accordance with the legends thereon; and

FIGURE 8 is similar to FIGURES 1 through 7 except that no photomicrographs are included therein.

In accordance with the teachings of our invention, the notch impact properties of mild steel can be markedly improved by a simple heat treatment. Both aluminum killed and rimmed steels are susceptible to improvement but the treatment is more effective for killed steels. The treatment has little or no effect on the microstructure as such. The treatment of our invention is effective for mild steels containing more than .04% and less than .15% carbon. A mild steel as understood herein is a low carbon steel containing no alloying ingredients other than manganese, silicon or aluminum and residual amounts of other elements. The maximum of the two elements mentioned are 1.5% manganese and .50% silicon.

We have discovered that the impact resistance of rimmed or aluminum killed steels containing less than about 0.15% and preferably over about .04% carbon is improved by a heat treatment in the range between the  $A_{e1}$  and about 1400° F., i.e. in the lower part of the alpha plus gamma field. The advantage gained does not depend upon the previous hot rolling or prior austenitizing temperature, which can be in the range 1600 to 2200° F. Furthermore, it does not depend upon the procedure used to attain the heat-treating temperature. The steel either may be air cooled from the austenitizing or hot-rolling temperature and then reheated to the heat-treating temperature, or it may be cooled directly from the austenitizing or hot-rolling temperature to the heat-treating temperature. Following the heat treatment, the steel may be air cooled. The advantage gained depends upon the length of the treatment in the alpha plus gamma region, up to about 24 hours.

2

Reference will be made to the following steels in illustrating the teachings of our invention:

|     | C   | Mn  | P    | S    | Si   | Al   |
|-----|-----|-----|------|------|------|------|
| 5 A | .10 | .41 | .011 | .024 | .01  | .001 |
| B   | .08 | .43 | .010 | .019 | —    | .003 |
| C   | .10 | .43 | .010 | .025 | .01  | .047 |
| D   | .10 | .43 | .011 | .024 | —    | .055 |
| E   | .19 | .82 | .010 | .019 | .16  | .029 |
| F   | .19 | .81 | .012 | .019 | .16  | .076 |
| G   | .23 | .54 | .013 | .028 | —    | .000 |
| H   | .16 | .99 | .018 | .028 | .038 | —    |
| I   | .21 | .72 | .028 | .039 | .20  | .024 |

As shown in FIGURE 1, the V-notch Charpy impact transition temperature of steel A, a rimmed 0.10% carbon steel was found to be about 80° F. after air cooling from 2100° F. When this steel was heated to 2100° F., quenched to 1350° F., held 24 hours, then air cooled, the V-notch Charpy impact transition temperature was reduced to about 55° F. In this and the other figures, the transition temperature is taken as the temperature at which the energy absorbed is half the difference between the maximum and minimum values observed. All photomicrographs are at a magnification of 100 diameters.

As shown in FIGURE 2, steel B, a steel similar to steel A, was heated to 1600° F., quenched to 1350° F., held 10 minutes, then air cooled reducing the V-notch Charpy transition temperature to about 55° F. When held 24 hours at 1350° F., the transition temperature was further reduced to about 20° F.

FIGURE 3 shows that the V-notch Charpy impact transition temperature for steel C, an aluminum-killed, 0.10% carbon steel, was about 90° F. after air cooling from 2100° F., about 45° F. after holding 2 hours at 1350° F., and about 18° F. after holding 24 hours at 1350° F. As shown by the photomicrographs of FIGURE 3, little change in microstructure or hardness accompanied this change in impact resistance.

The impact transition temperature of steel C referred to in FIGURE 3 was about -14° F. after austenitizing at 1600° F., quenching to 1350° F., holding 100 minutes, and air cooling. As shown in FIGURE 4, increasing the length of time at 1350° F. to 24 hours changed the impact transition temperature to -62° F. without significantly changing hardness or grain size.

The impact transition temperature of steel D, a 0.10% carbon aluminum-killed steel, normalized at 1650° F. was about -7° F. As is shown in FIGURE 5, reheating to 1350° F. and holding 24 hours caused the transition temperature to drop to -45° F. A similar, although smaller, effect was noted for a 0.10% carbon rimmed steel.

In both rimmed, steel B, and killed, steel D, 0.10% carbon steels, the notch impact behavior was not improved by quenching to 1450° F. and holding for various periods as shown in FIGURE 6. When the steels were quenched to 1300° F. and held, the impact properties deteriorated with time due to increase of ferrite grain size and spheroidization of carbides as shown in FIGURE 7. To prevent such microstructural changes and the resulting deterioration of impact properties, it is necessary for the lower limit of the heat-treating range to be above the  $A_{e1}$  temperature, which is about 1330° F. in the 0.10% carbon steels used. The upper limit is about 1400° F. A minimum time of about 10 minutes is required and the improvement increases with increasing time, the practical limit being about 24 hours.

In steels containing 0.16% carbon, or more, no improvement in impact properties was produced by reheating to the alpha plus gamma region after normalizing, or by quenching to this temperature range after austenitizing. This is shown for steel H in FIGURE 8. None of steels E through I responded favorably to the treatment of the

invention which is effective only in steels containing less than 0.15% carbon and preferably in the neighborhood of 0.1% carbon.

While we have shown and described several specific embodiments of our invention, it will be understood that these embodiments are merely for the purpose of illustration and description and that various other forms may be devised within the scope of our invention, as defined in the appended claims.

We claim:

1. A method of lowering the notch impact transition temperature of mild steel containing less than .15% carbon comprising quenching the steel from an austenitizing temperature to above the  $Ae_1$  temperature thereof and below about 1400° F., holding within such range for at least 10 minutes and air cooling.

2. A method of lowering the notch impact transition temperature of mild steel containing less than .15% carbon comprising quenching the steel from an austenitizing temperature to above the  $Ae_1$  temperature thereof and below about 1400° F., holding within such range for between 10 minutes and about 24 hours and air cooling.

3. A method of lowering the notch impact transition temperature of mild steel containing less than .15% carbon comprising quenching the steel from an austenitizing temperature to about 1350° F., holding at such temperature for at least about 10 minutes and air cooling.

4. A method of lowering the notch impact transition temperature of mild steel containing less than .15% carbon comprising quenching the steel from an austenitizing temperature to about 1350° F., holding at such temperature for between 100 minutes and about 24 hours and air cooling.

5. A method of lowering the notch impact transition temperature of mild steel containing less than .15% carbon comprising heating the steel to above the  $Ae_1$  temperature thereof and below about 1400° F., holding within such range for at least 10 minutes and cooling said steel from

said temperature without producing any substantial change in hardness or microstructure.

6. A method of lowering the notch impact transition temperature of mild steel containing less than .15% carbon comprising heating the steel to above the  $Ae_1$  temperature thereof and below about 1400° F., and holding within such range for between 10 minutes and about 24 hours and cooling said steel from said temperature without producing any substantial change in hardness or microstructure.

7. A method of lowering the notch impact transition temperature of mild steel containing less than .15% carbon comprising heating the steel to about 1350° F., holding at such temperature for at least about 10 minutes and cooling said steel from said temperature without producing any substantial change in hardness or microstructure.

8. A method of lowering the notch impact transition temperature of mild steel containing less than .15% carbon comprising heating the steel to about 1350° F., holding at such temperature for between 10 minutes and 24 hours and cooling said steel from said temperature without producing any substantial change in hardness or microstructure.

9. A method of lowering the notch impact transition temperature of aluminum-killed mild steel containing about .10% carbon comprising quenching the steel from about 1600° F. to about 1350° F., holding at such temperature for at least 100 minutes and cooling said steel from said temperature without producing any substantial change in hardness or microstructure.

#### References Cited in the file of this patent

Stoughton et al.: "Engineering Metallurgy," copyright 1953 by McGraw-Hill Book Co., pages 174 and 189 relied upon. Lib. of Congress call number 53-5559.

Iron and Steel Institute 1920, No. 11; vol. CII, Honda et al., p. 266 relied upon.

UNITED STATES PATENT OFFICE  
CERTIFICATE OF CORRECTION

Patent No. 3,062,693

November 6, 1962

Stephen B. Hudak et al.

It is hereby certified that error appears in the above numbered patent requiring correction and that the said Letters Patent should read as corrected below.

Column 4, line 6, after "1400° F.," strike out "and";  
line 34, for "pages 174 and 189" read -- pages 17, 174, 175  
and 189 --.

Signed and sealed this 16th day of April 1963.

(SEAL)

Attest:

ERNEST W. SWIDER  
Attesting Officer

DAVID L. LADD  
Commissioner of Patents